

Dec. 14, 1948.

R. L. MANEGOLD ET AL

2,456,136

ART OF SINTERING ORES

Filed April 20, 1945

FIG. 3.



FIG. 4.



FIG. 2.



FIG. 1.



INVENTORS

R. L. Manegold  
BY  
D. H. Wynnner  
Lieber & Lieber  
ATTORNEYS.

## UNITED STATES PATENT OFFICE

2,456,136

## ART OF SINTERING ORES

Robert L. Manegold, Shorewood, and Ira H. Wynne, Milwaukee, Wis., assignors to Dings Magnetic Separator Co., Milwaukee, Wis., a corporation of Wisconsin

Application April 20, 1945, Serial No. 589,412

3 Claims. (Cl. 75—5)

1

Our invention relates in general to improvements in the art of sintering ore, and relates more specifically to an improved method of and apparatus for sintering various types of ore with the aid of magnetism or magnetic influence.

The primary object of the present invention is to provide various improvements in the art of sintering ore, whereby such treatment may be most economically and efficiently effected without loss of valuable substances.

It is common practice in the art of metallurgy, to sinter or fuse finely divided ore particles into larger masses or lumps, after the ore has been concentrated and before the concentrates are charged into the smelters, in order to prevent undesirable ore dust losses. Likewise, it is common practice to sinter or fuse blast furnace flue dust before charging into the smelters. These sintering operations are usually carried on either with batch or continuous methods, by first mixing proper proportions of the ore, fuel and water into a homogeneous mass, by thereafter depositing a bed of the mixture upon either a fixed or a travelling grate, and by finally igniting the fuel and inducing a flow of combustion supporting air through the bed of material until the fuel has been consumed and the ore particles are nodulized. The air flow through the charges resting upon the grate bars is ordinarily produced by suction pressure established beneath the grate, and the sintered ore is subsequently deposited from the sintering grate upon a grizzly for eventual delivery to the smelters.

With these prior sintering methods, it is necessary to space the grate bars apart sufficiently to prevent the fine ore particles from being sucked freely through the grate openings, and the finer the ore the closer the bar spacing must be. As the grate openings are reduced in size, greater suction is required to provide sufficient volume of fresh air, and increased suction means increased power consumption and cost; and if the bars are spaced apart farther in order to eliminate such increased suction, greater quantities of valuable ore are drawn through the openings and are lost or must be returned. It is therefore most desirable to maintain the grate openings as large as possible in order to reduce the suction effort to a minimum, and to positively prevent free passage of fine material through these large openings.

We have discovered that these desirable results may be most effectively accomplished with the aid of magnetism, when sintering either magnetic or non-magnetic ores, by simply properly magnetizing the individual grate bars in a manner

2

whereby the magnetic fields created between adjacent bars will restrain the particles from being sucked out of the bed through the large grate openings. In the case of magnetic ores, the ore particles themselves may be magnetized in order to flocculate the mass and to assist in pelletizing the ore preparatory to sintering; and in the case of non-magnetic ores, the homogeneous batches may be mixed with magnetic blast furnace flue dust or other relatively fine magnetic material which may be pre-magnetized so as to produce a desirable degree of flocculation and pelletization of the ore in the charges being treated.

It is therefore a more specific object of our present invention to provide a new and useful process of sintering finely divided ore particles with minimum power consumption and with least loss of material, by properly magnetizing the bed supporting grate bars so as to permit free passage of gas while preventing undesirable escape of ore particles through the grate openings.

Another specific object of the invention is to provide an improved method of treating finely divided charges of ore and other materials preparatory to sintering the ore, by pre-magnetizing either the ore particles themselves, or finely divided particles of other material mixed with the ore, so as to flocculate the entire mass and to thereby facilitate the passage of combustion supporting air through the bed being treated.

A further specific object of this invention is to provide an improved grate for effecting most efficient and economical sintering of ore beds disposed thereon, and which is readily applicable to either batch or continuous ore sintering assemblies.

Still another specific object of our invention is to provide an improved magnetized ferrous grate bar assemblage especially adapted for the sintering of finely divided ore mixed with fuel and water to produce a homogeneous mass or mixture which is subject to ignition and penetration by combustion supporting air.

An additional specific object of the present invention is to provide a simple, compact and highly efficient ore sintering machine of the type comprising a series of horizontal parallel ore and fuel supporting grate bars through the separating spaces of which air is adapted to be drawn by suction from beneath the bar series.

These and other specific objects and advantages of the invention will be apparent from the following detailed description.

A clear conception of the features constituting our present improvement, and of the construc-

tion and mode of operating machines when carrying on our new method, may be had by referring to the drawing accompanying and forming a part of this specification wherein like reference characters designate the same or similar parts in the various views.

Fig. 1 is a diagrammatic side elevation of a fragment of an ore sintering assemblage, looking toward the ends of the ore bed supporting grate bars;

Fig. 2 is a similarly diagrammatic top view of the grate bars embodied in the assemblage of Fig. 1;

Fig. 3 is an enlarged transverse vertical section through an adjacent pair of permanently magnetized grate bars, illustrating the magnetic fields normally produced by these bars; and

Fig. 4 is a similarly enlarged transverse vertical section through an adjacent pair of electrically energized magnetic grate bars, also showing the magnetic fields normally produced thereby.

While our invention has been shown and described herein as being especially adapted for application to an ore sintering assemblage of the suction type, it is not our desire or intention to unnecessarily limit the scope or utility of the improvement for analogous purposes, and the designations N and S appearing on the drawings indicate positive and negative polarity respectively.

In accordance with our present invention, and as shown in the drawing, we provide a grate for an ore sintering machine or the like, comprising a series of elongated parallel bars 6, 7, which may be either permanently magnetized or magnetized by induction, so as to create fields of magnetic influence between the successive or alternate adjacent bars of the grate. As shown, the bars 6, 7 are preferably so magnetized that the upper and lower portions of the successive bars 6, 7 are of opposite polarity, that is, the upper portions of the bars 6 are positively charged and the lower portions thereof are negatively charged, while the upper portions of the intervening bars 7 are negatively charged and the lower portions thereof are positively charged. By thus magnetizing the bars 6, 7 of the series, relatively strong magnetic fields are created across the upper and lower portions of the spaces 8 separating the adjacent grate bars, and these fields of magnetic influence extend throughout the entire length of the bars or entirely across the grate.

When permanently magnetized grate bars 6, 7 are utilized as in Figs. 1, 2 and 3, it is preferable to form these bars of metal such as "Alnico" having highly magnetic characteristics. This metal consists of a compound of aluminum, nickel, cobalt and iron, and is susceptible of powerful magnetization for indefinite duration. However, the grate bars need not be permanently magnetized and may in fact be magnetized by induction as illustrated in Fig. 4, wherein the bars 6', 7' are properly magnetized with the aid of electrically energized coils 9, 10 respectively longitudinally embracing the medial portions of the bars 6', 7'. These coils 9, 10 may be embedded in recesses 11 formed in the bars 6', 7', and may be energized in any convenient and well known manner.

When the grate bars 6, 7 have been properly assembled and magnetized they provide a grate for supporting a bed of homogeneous mixture 12 of finely divided ore, sufficient fuel to effect nodulation of the ore, and water in sufficient quantities to hold the solid particles together. This mixture bed 12 may be caused to rest upon the

grate and may be of any desired depth, and the bed 12 is preferably constantly supplied with combustion supporting fresh air which may be drawn through the mass and through the grate openings 8 by suction created in the zone beneath the bars 6, 7 in a well known manner and as indicated by the arrows in Figs. 3 and 4.

If the ore to be treated is of a magnetic type, it may be found advantageous in order to loosen or flocculate the bed 12, to pre-magnetize the ore particles before they are subjected to sintering, and this may also be done in any convenient and well known manner. In case the ore is not inherently magnetic, some degree of flocculation of the charge may be attained by including in the mixture a suitable quantity of pre-charged magnetic pulverulent material such as blast furnace flue dust or magnetite which is ordinarily available in metallurgical plants. Such pre-magnetizing of the charges besides loosening or floculating the beds 12 also assists in pelletizing the ore prior to sintering and permits freer passage of air and gases therethrough, thus facilitating more rapid and less restrained flow of the gases toward the discharge spaces 8.

While the improved method of sintering ore in accordance with our present invention should be apparent from the foregoing description, a short résumé of the process will be repeated. After the grate bars have been properly magnetized, constructed and assembled so as to produce relatively wide and unobstructed intervening spaces 8, and the mixture of ore, fuel and water has been properly prepared, successive charges or beds 12 of the mixture may be deposited upon the assembled grate, whereupon the fuel should be ignited and suction should be created beneath the grate and bed. The burning fuel in the charges will evaporate the water and nodulize or fuse the fine ore particles, and fresh air will be drawn into the top of the beds while the gases of combustion will be constantly withdrawn through the spaces 8 by suction.

During this sintering performance or operation, the magnetized grate bars will create relatively strong fields of magnetic influence above and below each complementary pair of adjacent bars as clearly shown in Figs. 3 and 4, and these magnetized zones or fields will cause some of the magnetic particles of the charges to assume gap bridging groups or patterns spanning the large spaces 8 at their lower and upper ends. This bridging action places a relatively loose barrier across each end of each space 8, which while permitting relatively free flow of gases therethrough, positively prevents ore particles from dropping out of the mass of mixture. When the fuel has been completely consumed, the sintering or nodulation will have been completed, and successive charges may thus be quickly and effectively treated with the aid of minimum suction effort and without losing valuable ore.

It is a well known fact that permanent magnets when subjected to excessively high temperatures, rapidly lose their magnetism, but that a moderate increase in temperature improves the magnetic properties. It is also a well known fact that the sintering of ores is accomplished at relatively high temperatures which if directly applied to a permanent magnet, might undesirably affect the magnetization. We have found, however, that with our improved method, the extreme sintering temperatures do not materially affect permanently magnetized bars 6, 7 since these bars are adapted to rapidly radiate the heat into the

spaces 8 and into the suction zone, and that the temperatures to which these bars are actually subjected during sintering are not sufficient to undesirably affect the magnetization thereof. We have also found that by magnetizing the grate bars, the spaces 8 can be made considerably larger than is possible without utilizing the present improvements, while still avoiding loss of valuable ore particles. It is also noteworthy that when the bridges of magnetic material have been produced, they remain in place and provide a cushion for the bed 12, and in cases where the ore has non-magnetic characteristics, the improved results may be obtained either by applying magnetic pulverulent material to the charges, or by initially placing a layer of magnetic particles near the magnetic bars so as to produce the bridging patterns before the charges are actually applied to the grate. Our invention has in fact proven highly successful in actual use and has established the fact that magnetization of the grate bars will permit more rapid and effective sintering at minimum cost and without the loss of valuable product. By pre-magnetizing magnetic ores, the charges of material being sintered may also be maintained in loosened and flocculated condition, thereby facilitating the impregnation of the charges with fresh combustion supporting air; and it has been found that when either magnetic or non-magnetic ore is being sintered, there is an intense magnetic zone produced around the bars, and this magnetic action loosens and flocculates the ore in the vicinity of the grate to a depth of several inches or more.

It should be understood that it is not desired to limit this invention to the exact details of construction or to the precise steps of the method, herein shown and described, for various modifications within the scope of the appended claims may occur to persons skilled in the art.

We claim:

1. The method of sintering a static bed of mixed magnetic ore and fuel particles resting upon a grate having supporting bars spaced apart sufficiently to normally permit particles of the mixture to gravitate freely through the spaces, which comprises, magnetizing and maintaining the bars constantly magnetized with sufficient intensity to cause the magnetic particles to loosely bridge each space with bridges sufficiently dense to prevent particles of the mixture from falling

through the spaces, and igniting the fuel particles to sinter the mixture and continuing the sintering operation by passing combustion air and gases through the bed and spaces.

- 5 2. The method of sintering a static bed of mixed magnetic ore and fuel particles resting upon a grate having supporting bars spaced apart sufficiently to normally permit particles of the mixture to gravitate freely through the spaces, which comprises, individually magnetizing and maintaining each bar constantly magnetized with sufficient intensity to cause the magnetic particles to loosely bridge each space with upper and lower bridges sufficiently dense to prevent particles of the mixture from falling through the spaces, igniting the fuel particles to sinter the mixture and continuing the sintering operation by admitting combustion air to the bed, and discharging the gases of combustion downwardly through the bridges and spaces.
- 10 3. A grate assemblage for sintering a static bed resting thereon and composed of mixed magnetic ore and fuel particles, which comprises, a series of bed supporting bars separated by elongated structurally unobstructed spaces of sufficient width to normally permit most of the particles of the bed to gravitate freely therethrough, said bars being individually constantly magnetized with sufficient intensity to cause magnetic particles of the mixture to bridge the upper and lower portion of each space with bridges sufficiently dense to support the entire bed above the grate and to prevent any particles of the mixture from falling through said spaces while permitting free flow of gases through the latter.
- 15 30

ROBERT L. MANEGOLD.  
IRA H. WYNNE.

#### REFERENCES CITED

- 40 The following references are of record in the file of this patent:

#### UNITED STATES PATENTS

| Number       | Name | Date          |
|--------------|------|---------------|
| 45 2,048,111 | Gahl | July 21, 1936 |
| 2,048,113    | Gahl | July 21, 1936 |

#### OTHER REFERENCES

- 50 "Electromagnetic Devices," by Herbert C. Roters, 1941, pages 45 and 46.